

K. NOMI.

UTILIZATION OF PETROLEUM PITCH.

APPLICATION FILED JAN. 22, 1918.

1,386,945.

Patented Aug. 9, 1921.



Lloyd R. Cornwall  
witness.

83

J. R. Kerslake.

Attorney

# UNITED STATES PATENT OFFICE.

KONOSUKE NOMI, OF KITATOSHIMA-GUN, JAPAN.

## UTILIZATION OF PETROLEUM-PITCH.

1,386,945.

Specification of Letters Patent.

Patented Aug. 9, 1921.

Application filed January 22, 1918. Serial No. 213,124.

To all whom it may concern:

Be it known that I, KONOSUKE Nomi, a subject of the Emperor of Japan, residing at No. 1987 Sugauro-Mura, Kitatoshima-gu, Tokyo Province, Japan, have invented certain new and useful Improvements in the Utilization of Petroleum-Pitch, of which the following is a specification.

This invention relates to the utilization of petroleum pitch or more particularly to a method of obtaining coke, aromatic volatile oil and gas (the gas consisting largely of hydrogen), by charging petroleum pitch into a retort made of cast iron or of fire clay, heating it to the temperature of about 500° to 600° C. to carry out destructive distillation. The object of this invention is to obtain these products cheaply.

The petroleum pitch preferably employed in the process, is a by-product of refining petroleum oils containing olefins in relatively large quantities. The melting point of the material varies more or less, depending upon the exact mode of production. A particular sample melted at 80° C., and this may be considered as an average melting point.

In carrying this invention into practice, a suitable retort made of cast iron or of fire clay is employed. After charging this retort with a suitable quantity of petroleum pitch, this is heated gradually. When the charge is heated to about 400° C., (which may require about two hours) it begins slowly to decompose, which operation becomes most efficient when the temperature reaches about 400 to 550° C., say about 500° C. During this operation, a pressure of about 4 or 5 pounds per square inch above atmospheric is preferably maintained in the retort. The mass in the retort is then heated further, care being taken that the temperature does not exceed 600° C., the decomposition into the products above mentioned is completed. During this latter step, a pressure slightly below atmospheric is used, a suction of 1 to 2 inches being preferred. The retort will contain coke of the best quality with only a very small percentage of impurities. The distillate is collected in a suitable receiver by passing the volatile products through a condenser which is connected to the retort. The gas is led into a tank through an iron pipe connected to the condenser.

The amounts of products according to this

invention are roughly given in the following table (per 1000 kgs. of the petroleum pitch);

|                                                            |    |
|------------------------------------------------------------|----|
| Coke, about 450 kilograms.                                 | 60 |
| Distillate, about 250 kilograms.                           |    |
| Gas consisting largely of hydrogen, about 6000 cubic feet. |    |

In a particular test run of the process, the products produced were examined with the following results:

### (a) Composition of coke.

|                  |                |
|------------------|----------------|
| H <sub>2</sub> O | 1.74%          |
| Volatile part    | 3.74%          |
| Carbon part      | 92.06%         |
| S                | 1.00%          |
| P                | Trace          |
| Ash              | 1.50%          |
| Calorific power  | 8743 calories. |

### (b) Composition of gas.

|                    |       |
|--------------------|-------|
| H                  | 60.1% |
| O                  | 1.5%  |
| CO                 | 0.9%  |
| CO <sub>2</sub>    | 0.7%  |
| CH <sub>4</sub>    | 18.5% |
| Other hydrocarbons | 18.3% |

### (c) Sp. gr. of volatile oil (fraction distilling between 50° C. and 110° C.), 0.852.

This liquid consists largely of olefin hydrocarbons, but contains some (say 3%, more or less) of aromatic hydrocarbons, toluol, benzol, etc.

The coke remaining in the retort contains only a minute quantity of sulfur and ash so that it has not only a higher calorific power than ordinary coke, but also is very suitable for raw material for smelting iron, or for producing graphite carbon for electric purpose.

The distillate collected in the receiver contains about 60% of volatile oil (having boiling point of under 150° C.), which, therefore, is separated from the heavier oils by fractional distillation, preferably at not greatly exceeding atmospheric pressure. The residual oil is mixed with about ten times its weight of molten pitch. This mixture is thereafter charged into the retort and the distilling operation is repeated as before, forming the second run. The volatile oil obtained in this second run consists chiefly of aromatic hydrocarbons, and not only can be used as a solvent for rubber,

fats or the like, but also can replace petroleum-benzin, or otherwise employed as a volatile oil.

The gas produced as a by-product in the dry distillation will amount to about 6000 cubic feet by volume, per one ton of the pitch. A part of this gas can be burned to supply the amount of heat required for carrying out this process and, therefore, no external fuel is needed. This gas contains about 55 to 60% hydrogen, while carbon monoxide and carbon dioxide amount to less than 2%. Therefore, the gas can be used for oil hardening after comparatively simple purification treatment.

Briefly, this invention enables one to directly obtain coke of good quality from cheap petroleum pitch. Moreover, according to this invention the distillate is subjected to fractional distillation to obtain volatile oil, the residue of which operation can be again charged into the retort, with more pitch, to produce coke and volatile oil, and at the same time gas consisting chiefly of hydrogen being produced as a by-product. Therefore, these products, viz, coke, volatile oil and the gas can be very cheaply obtained of comparatively good quality.

In the accompanying drawings, which shows one example of apparatus suitable for carrying this invention into practice, Figure 1, is a diagrammatic elevation of an apparatus for heating the petroleum pitch in a retort, together with its connections. Fig. 2 is a diagrammatic elevation, partly in section, of an apparatus for subjecting the distillate to fractional distillation. Fig. 3 is a plan view, partly in section, of the apparatus shown in Fig. 2.

In Fig. 1, 1 is a retort furnace having for example, three horizontal retorts 2, each provided with an exit pipe 3, leading to a hydraulic main 4. 5 is a tank for collecting gases escaping from the retort. 6 is another tank or receiver for collecting the distillate, which is condensed in the hydraulic main 4, which acts as a condenser.

In Figs. 2 and 3, 15 is a still for fractional distillation, which is to be charged with the distillate from tank 6. The material in 15

is distilled by heating the same sufficiently to cause distillation. If the pressure rises a little above atmospheric, no particular harm is done. The vapor coming from the still is passed through a pipe 16, first partially cooled and condensed in a condenser 17, the condensate being collected in a receiver 18. A second part of the vapor which is not condensed in 17, is passed through a pipe 19, condensed in the second condenser 20 and is collected in a receiver 21. The condensate is drawn off from the receivers and may be mixed with a new charge of petroleum pitch as described. Or, if desired, this condensate may be returned to the still by a return pipe 22, which may be provided with a cock 23 for the purpose. The volatile oil, which is not condensed in the tanks 17 and 20, is finally condensed in a condenser in 24. 25 is a charging pipe for the still. 26 is a safety valve.

The steps of the process may be carried out at about atmospheric pressure.

I claim:

1. The process herein described, which comprises destructively distilling at about 500 to 600° C. a mixture of petroleum pitch and the heavy components of the oil produced in the destructive distillation of petroleum pitch, whereby an oil containing a large percentage of aromatic hydrocarbons, coke and gas are produced.

2. Process of producing coke, volatile oil and gas containing hydrogen, which comprises charging a suitable retort with petroleum pitch, then heating it up to about 500° to 600° C., and collecting the products, fractionally distilling the volatile oil obtained, and mixing the heavier fraction thereof with an additional quantity of the petroleum pitch, and heating said mixture to about 500° to 600° C., and collecting the products.

In testimony whereof I have hereunto set my hand in presence of two subscribing witnesses.

KONOSUKE NOMI. [L. S.]

Witnesses:

HENRY B. HITCHCOCK,  
JORG BODCHIGADJ.